

## UNITED STATES PATENT OFFICE

1,976,873

## REMOVING SOLVENTS FROM PLASTIC COLLOIDS

Harry P. Bassett, Cynthiana, Ky.

No Drawing. Application June 26, 1931,  
Serial No. 547,191

7 Claims. (Cl. 18—51)

This invention relates to a process of removing solvents from semi-solid or plastic colloids and in its specific embodiment relates particularly to the removal of solvents from cellulose nitrate plastic compositions such as celluloid.

The principal object of this invention is to provide a simple and efficient process of removing solvents from plastic colloids whereby a product of superior quality is obtained and the removal of solvents is accomplished in a relatively short period as compared with the time required in similar processes heretofore generally employed.

An important object of this invention is to provide a simple, rapid and efficient process of removing solvents from nitro-cotton or similar plastic compositions which is substantially free from the disadvantages commonly encountered in the processes heretofore generally employed for similar purposes.

A further object of this invention is to provide an improved process of preparing celluloid or other plastic sheets which are particularly adapted for use in making shatter-proof glass.

25 Other objects and advantages of the invention will become apparent during the course of the following description.

I have discovered a simple process for removing solvents from freshly formed or partially finished plastic colloids such as vulcanized fiber, celluloid, and the like, which process not only is particularly effective in removing the solvents but produces finished products of superior qualities and appearance. While, as suggested, the 35 process is applicable for use for removing solvents such as zinc chloride from plastic compositions such as vulcanized fiber, the invention is particularly adapted for application in the removal of solvents from cellulose nitrate plastic 40 compositions, particularly celluloid. The process is based on my discovery that solvents may be removed from plastic colloids without harm to the quality or color of the final product by exposing such colloids to an atmosphere of the 45 vapor of a nonsolvent of the colloid which is miscible with the solvent in the colloid and thereafter heating the colloid in a dryer at gradually increasing temperatures between the approximate limits of 100° F. and 160° F. In the preferred practice of the process the vapor bath or atmosphere to which the colloid is initially exposed contains a major proportion of the solvent-miscible nonsolvent of the colloid, the concentration of which in the atmosphere is reduced during the process, the heating of the

colloid in the manner above referred to being started after the first reduction of the concentration of the nonsolvent of the colloid and being further gradually decreased as the temperature is gradually increased.

I have found that water vapor may, for the purposes of greatest efficiency and economy, be employed as the nonsolvent of the colloid which is miscible with the solvent in the colloid. Accordingly, in preferred practice, I subject a freshly formed or partially finished plastic colloid to be treated to the action of an atmosphere of water vapor. While the percentage of the water vapor present in the vapor bath or atmosphere may be varied to a considerable extent, I have found that improved results are obtained if the water vapor is used in such amount that the relative humidity of the atmosphere in the vapor bath is about 70%, and preferably in the neighborhood of 76%. While various vapors or gases may be employed 75 as the diluting factor in the vapor bath, air is the obvious aeriform fluid to be employed for this purpose and since fully satisfactory results are obtained when air is employed, I recommend its use. Thus, in preferred practice the plastic colloid is 80 initially subjected to a vapor bath of air and water vapor, the relative humidity in which atmosphere is above 70% and preferably about 76%.

After subjecting the colloid to such an atmosphere for from several hours to several days, depending upon the nature, size, thickness, etc. of the colloid under treatment, the concentration of the water vapor in the bath is preferably reduced so that the relative humidity of the resulting atmosphere is materially lowered, say to 40%. 90 Thereafter, the content of water vapor is lowered again, preferably to such an extent that the resulting atmosphere will have a relative humidity of about 15%. Of course, the lowering of humidity may be more gradual than just indicated, if desired, but I have found that a more gradual reduction in the concentration of water vapor in the atmosphere is not necessary in general practice. Either after the original humidity of the vapor bath has been lowered, to say about 40%, or after the reduction of the humidity to the lowest point to which it is to be lowered (or at any intermediate point, for that matter), the colloid is heated to a temperature of say 100° F. and the temperature is gradually raised, over a period of 105 from several hours to several days, to a more elevated temperature which ordinarily should not exceed 160° F. As stated above, the temperature is gradually increased as the humidity of the vapor bath is gradually decreased. After the 110

completion of this treatment it will be found that the solvents present in the colloids are substantially removed and the products are in condition for general use.

5 Whereas, in accordance with the preferred embodiment of the invention, solvent is to be removed from cellulose ester colloids, the freshly formed articles which may be obtained either by slicing a block of the partially finished plastic 10 colloid or by extruding a plastic colloid mix, are suspended in a chamber which may conveniently be a drying chamber of conventional type for ageing or seasoning plastic colloid articles. In the initial stage of the process the vapor treating bath is introduced into the drier preferably by causing water vapor to enter from the bottom of the drier together with air. The drier should be provided with an outlet at the top so that there will be a current of the treating vapor 15 through the drier. I have found it convenient to employ a cold water spray at the inlet of the drier which may be controlled to regulate the humidity in the drier. As stated above, I prefer that the atmosphere to which the freshly 20 formed plastic colloids are initially exposed shall have a relative humidity preferably in excess of 70% and, for best commercial practice under ordinary conditions, about 76%. The temperature of the atmosphere in the initial treatment 25 of the articles may advantageously be normal atmospheric temperature. Such an atmosphere may be used for all thicknesses of articles in the initial treatment but the time of treatment with this atmosphere will be varied according to 30 the particular thickness of article. For example, in the case of a plastic colloid article having a gauge of 215, I prefer to leave the article in this atmosphere for about five days. On the sixth day the humidity in the drier is preferably reduced to about 40% and heated air is introduced 35 into the drier so that the temperature therein will be approximately from 100° to 104° F. On the seventh day, the humidity is dropped to about 15% and the temperature in the drier is raised to about 115° F. Thereafter, the temperature is raised gradually to 130° F. for the eighth day, to 150° F. for the ninth day, and to 40 160° F. for the tenth and eleventh days. At the end of this time, the stock is fully aged and 45 ready to be used.

50 As is apparent from the foregoing, a treatment for eleven days is sufficient for relatively thick celluloid articles. As articles of lesser thickness are treated, the time of treatment 55 may be correspondingly decreased. For example, with a 60 gauge plastic colloid article, I have found that complete ageing is obtained by treatment for approximately one day in a vapor bath of the characteristics set forth above at ordinary temperature, followed by a treatment 60 for about twelve hours at reduced humidity and a temperature of 100° F., subsequent treatment for twelve hours at 130° F., with treatment for one day at 160° F. as a final step. Of course, 65 the increase in temperature is preferably gradual and the decrease in humidity of the vapor bath is likewise gradual. However, some satisfactory measure of success may be obtained by initially reducing the humidity to the minimum degree 70 of humidity employed followed by the gradually increasing heat treatment.

75 While I have described in detail the preferred practice of my process it is to be understood that the details of procedure, such as the time of treatment, the vapor bath employed, and the

concentration of treating agent in the vapor bath, may be variously modified without departing from the spirit of the invention or the scope of the subjoined claims.

I claim:

1. The process of removing solvent from a cellulose ester plastic composition containing the same and containing a plasticizing agent which comprises treating such colloid in an atmosphere of water vapor, thereafter heating the thus treated colloid at gradually increasing temperatures between the approximate limits of 100° F. and 160° F., and gradually reducing the concentration of water vapor in the atmosphere surrounding said colloid during said heating. 80

2. The process of removing solvent from a cellulose ester plastic composition containing the same and containing a plasticizing agent which comprises exposing such colloid to an atmosphere of water vapor, the relative humidity of which is above 70, thereafter heating the thus treated colloid at gradually increasing temperatures between the approximate limits of 100° F. and 160° F., and gradually reducing the concentration of water vapor in the atmosphere surrounding said 90 colloid during said heating. 95

3. The process of removing solvent from a cellulose ester plastic composition containing the same and containing a plasticizing agent which comprises exposing such colloid to an atmosphere of water vapor, the relative humidity of which is above 70, gradually reducing the humidity of said atmosphere and, while the humidity is being reduced, heating the colloid at gradually increasing temperatures between the approximate limits of 100° F. and 160° F. 105

4. The process of removing solvent from a cellulose ester plastic composition containing the same and containing a plasticizing agent which comprises exposing such colloid to an atmosphere of water vapor, the relative humidity of which is approximately 76, gradually reducing the humidity and simultaneously heating the colloid at gradually increasing temperatures between the approximate limits of 100° F. and 160° F. 115

5. The process of removing solvent from a freshly formed cellulose nitrate plastic composition which comprises treating such composition with a bath of water vapor, thereafter heating the composition at gradually increasing temperatures between the approximate limits of 100° F. and 160° F., and gradually reducing the concentration of water vapor in the atmosphere surrounding said 120 composition during said heating. 125

6. The process of removing solvent from a freshly formed cellulose nitrate plastic composition which comprises exposing such composition to an atmosphere of water vapor, the relative humidity of which is above 70, and reducing the humidity of said atmosphere and heating the composition at gradually increasing temperatures between the approximate limits of 100° F. and 160° F. 130

7. The process of seasoning freshly formed cellulose ester plastic composition sheets containing a solvent and plasticizing agent which comprises exposing such sheets for a period of from several hours to several days to an atmosphere of water vapor, the relative humidity of which is approximately 76%, gradually reducing the humidity of said atmosphere, and heating the sheets over a 145 period of several days at gradually increasing temperatures between the approximate limits of 100° F. and 160° F. 140

HARRY P. BASSETT.

150